# EUROPEAN PATENT APPLICATION

(11) **EP 0 758 015 A1**
(43) Date of publication of application: **12.02.1997**
(21) Application number: 96305407.7
(22) Date of filing: 23.07.1996
(51) Int. Cl.: C10L 1/18

(54) **Icing inhibitors**

(30) Priority: 09.08.1995 GB 9516446
(71) Applicant: BP Chemicals Limited, London EC2M 7BA (GB)
(72) Inventor: Pacynko, Witold Franciszek, Hull, North Humberside HU12 8DS (GB)
(74) Representative: Krishnan, Suryanarayana Kalyana

(57) **Abstract**

This invention relates to an icing inhibitor for hydrocarbon fuels contaminated with water said icing inhibitor comprising a polyethyleneglycol monoalkyl ether of the generic formula: R-(OCH₂.CH₂)_{*n*}-OH wherein R is a C4-C6 alkyl group and *n* has a value from 3 to 8, said inhibitor being substantially free of components immiscible with said fuel and an aviation fuel system comprising a hydrocarbon fuel contaminated with water, and an ice inhibiting amount of a polyethyleneglycol monoalkyl ether which is preferably triethyleneglycol mono-n-butyl ether.

## Description

This invention relates to icing inhibitors for fuel systems and particularly to the use of such inhibitors in aviation fuels.

It is known that hydrocarbon fuels, especially aviation fuels contain small amounts of dissolved water. Such aviation fuel specifications normally permit from 70-120 ppm of water although the amount of dissolved water, and in some cases suspended water, may be much higher in hydrocarbon fuels in general. The water content usually varies with the source of the fuel or the refinery in which it is produced. The presence of water becomes problematical when modern jets fly at high altitudes. At relatively high altitudes, fuel tanks in jets encounter very low temperatures which in turn causes the water present in such fuels to come out of solution as small droplets and freeze into ice particles. Such ice particles can and do cause blockage of the fuel line filters with catastrophic results. This problem is alleviated in some cases by the use of on-line heaters. However, many aircraft and helicopters are not equipped with such on-line heaters. Known anti-freezes and deicers such as glycols cannot be used as such because they are substantially immiscible with the fuel. Thus, in the prior art such glycols have been used as a blend or admixture thereof with glycol ethers. One such formulation is described in GB-A-997906 in which the ice formation in the carburettor of internal combustion engines is prevented by adding to the gasoline between 0.02 and 0.05% by volume of gasoline, a mixture of (a) two or more gasoline soluble diols being an addition product of propylene oxide with propane diol-1,2 or (b) two or more gasoline soluble alkylene glycol ethers of a general formula R-(OCH₂-CH₂)_{*n*}-OH in which R denotes a methyl, propyl or butyl radical and n denotes 2 or 3, or (c) one or more of the diols (a) with one or more of the ethers (b). This publication states that the activity of the diols (a) is far above that of the individual diols, but is in general considerably increased by adding one or more alkylene glycol ethers according to their invention. Further this publication states that the good solvent properties of the diol and/or alkylene glycol mixtures permit the addition of diols known as outstanding freezing point depressant compounds but hitherto not usable as anti-icing additives by reason of their insolubility in gasoline. Butyl triglycol ethers are only mentioned in this publication when used as a mixture thereof with and as a solubilising agent for diols which are used as the freezing point depressants. It is to be noted that in this publication there is no performance data on the anti-icing agents at temperatures below 0°C. Similarly, US-A-3925030 describes an anti-icing composition useful as a gasoline additive which comprises (a) 30-90 wt % of a gasoline soluble organic compound of the formula Z-OH which represents an alcohol, a glycol or a glycol ether in which Z has 4-180 carbon atoms and (b) and 10-70 wt% of a gasoline soluble polycarboxy hydrocarbon having 25-75 carbon atoms. In this latter publication, component (b) represents an anti-stalling additive for the engine and is said to have no anti-icing characteristics. Again, GB-A-1124193 describes an additive for hydrocarbon fuels, especially aviation fuels comprising glycol ethers, especially methyl and ethyl ethers of diethylene glycol (also known as diglycol) and the methyl ether is said to be preferred. However, conventional glycols and glycol ethers such as methyl glycol ether (MGE) and methyl diglycol ether (MDGE), when used in fuels with which they are miscible, partition into the water phase and - like the diols - act by depressing the freezing point. However, such glycol ethers are also known reprotoxins. MGE is a Category 2 Reprotoxin whereas MDGE is a Category 3 Reprotoxin and are hence regarded undesirable. The main hazards with these glycol ethers occur during contact with the operatives whilst emptying either fuel or storage tanks, or, during subsequent waste water treatment/disposal. In view of this, industry has been forced to seek alternative, less hazardous icing inhibitors.

It has now been found that the above problems can be solved by the use of icing inhibitors which do not act by depressing the freezing point but act by preventing water from separating out of the fuel at relatively low temperatures, ie by reducing the dew point of the fuel.

Accordingly, the present invention is an icing inhibitor for hydrocarbon fuels contaminated with water said icing inhibitor comprising a polyethyleneglycol monoalkyl ether of the generic formula:

R-(OCH₂.CH₂)_{*n*}-OH (I)

wherein R is a C4-C6 alkyl group and *n* has a value from 3 to 8, said inhibitor being substantially free of components immiscible with said fuel.

According to a further embodiment, the present invention is an aviation fuel system contaminated with water, and comprising an icing inhibitor, said icing inhibitor comprising a polyethyleneglycol monoalkyl ether (I) and being substantially free of components immiscible with said fuel.

According to a yet another embodiment, the present invention is an aviation fuel system comprising an ice inhibiting amount of a polyethyleneglycol monoalkyl ether (I).

The hydrocarbon fuels which may be treated in the above manner are suitably conventional aviation and jet engine fuels which comprise a blend of hydrocarbons boiling suitably in the range from about 37°C to about 375°C, preferably in the range from 90°C to 330°C, such as eg gas oils, kerosines and gasoline. Fuels with varying degrees of aromatic content ranging from 5 to 90 percent liquid volume of aromatics which are used for operating turbo aircraft engines can be treated according to the present invention. Specific examples of the fuels which may be treated according to the invention are the commercially sold fuels including *inter alia* those sold under the names JET A, JET A-1, AVTUR, JP-3, JP-4, JP-5, JP-8 and jet kerosine.

Thus, the polyethyleneglycol monoalkyl ether (I) (hereafter referred to as "PGME" for convenience) is suitably an ether in which the alkyl group R is a C4 alkyl group and the *n* has a value of 3-4. The alkyl group R is preferably an n-butyl group. Thus, the PGME is most preferably triethyleneglycol mono-n-butyl ether (also known as butyl triglycol ether and hence will hereafter referred to as "n-BTGE" for convenience).

The PGME can be used as a single ether or as an admixture thereof with other alkyl mono-, alkyl di- or alkyl polyglycol ethers. Such an admixture suitably contains a butyl triglycol ether, preferably n-BTGE which is most preferably present as the major component. Suitable examples glycol ethers that may be present in the PGME in addition to butyl triglycol ethers include *inter alia* alkyl di-, alkyl tetra- and/or alkyl penta-glycol ethers. An icing inhibitor comprising a mixture of n-BTGE and an alkyl tetra-glycol ether such as n-butyl tetra ethyleneglycol ether is most preferred.

The amount of icing inhibitor used is suitably in the range from 0.01 to 1% by weight of the hydrocarbon fuel, preferably from 0.1 to 0.5% by weight, most preferably from 0.1 to 0.2% by weight. Where n-BTGE is admixed with other alkyl glycol ethers, n-BTGE is present in such admixtures in an amount of at least 50% by weight of the total admixture, suitably above 60% by weight preferably above 70% by weight. One such composition which:
a. is formed as a by-product stream during the manufacture of alkylene oxides,
b. is commercially available and
c. can be used as an icing inhibitor
and will hereafter be identified as "Solvent 14" comprises the following components in approximate weight %:

| | |
|---|---|
| n-Butyl triglycol ether - | 75 |
| n-Butyl diglycol ether - | 2.5 |
| n-Butyl tetraglycol ether - | 19.0 |
| n-Butyl pentaglycol ether - | 2.0 |

Such a composition can be readily used without any need to separate the individual components.

A surprising feature of the present invention is the ability of the icing inhibitor according to the present invention to reduce the dew point of aviation fuel to prevent icing. An even more striking aspect of the icing inhibitor according to the present invention is its superior performance at the same concentrations when compared with convention glycol ether inhibitors. This is surprising because hitherto, butyl triglycol ethers had been regarded as an inferior icing inhibitor when compared with glycols and other conventional glycol ethers and which all relied on the ability of such glycols and ethers to act as a freezing point depressant. It was not recognised hitherto that the same effect of icing inhibition can be achieved by reducing the dew point of the fuel thereby preventing the separation/precipitation of water droplets from the fuel and thereby avoiding the need to depress the freezing point of water. PGME in general n-BTGE in particular achieves this with significant effect and prevents icing at considerably lower temperatures than would be possible with conventional freezing point depressants.

The present invention is further illustrated with reference to the following Examples:

Various glycol ethers were tested for their ability to reduce the dew point and their performance was compared with that of Solvent 14 (according to the present invention). The inhibitor was admixed in the concentrations specified in Tables 2 and 3 below with an aviation turbine fuel saturated with about 80 ppm of water and the dew point of the admixture measured by monitoring the temperature at which the fuel became cloudy. Aviation turbine fuels are generally a complex combination of hydrocarbons produced by the distillation of crude oil. They predominantly consist of hydrocarbons having C9-C16 hydrocarbons and the fuel used in these experiments had typical physical properties shown in Table 1 below:

**TABLE 1**

| Aviation Turbine Fuel | | |
|---|---|---|
| Property | Test Method | Data |
| Physical state | - | Liquid |
| Colour | - | yellow |
| Odour | - | kerosine-like |
| Density @ 15°C | ASTM 1298 | 751-840 kg/m³ |
| Boiling point range | ASTM 86 | 300°C maximum |
| Flash point (Abel) | ASTM 3828 | >38°C |
| Kinematic viscosity @ -20°C | ASTM445 | Approx. 8.0 mm²/s |

The following icing inhibitors were tested:
a. Solvent 14 composition (according to the invention)

| | |
|---|---|
| n-Butyl triglycol ether - | 75 % by weight |
| n-Butyl diglycol ether - | 2.5 % by weight |
| n-Butyl tetraglycol ether - | 19.0 % by weight |
| n-Butyl pentaglycol ether - | 2.0 % by weight |

b. Ethoxyethoxy ethanol (hereafter "EDGE")
c. Ethoxypropoxy propanol (hereafter "EDP")
d. Butoxy ethanol (hereafter "BGE")
e. Butoxyethoxy ethanol (hereafter "BDGE")
f. n-Butyl propylene glycol ether (hereafter "PnB")
g. n-Butyl dipropylene glycol ether(hereafter "dPnB")
h. t-Butyl propylene glycol ether (hereafter "PnBtert") The results achieved are tabulated Tables 2 and 3 below. Table 2 summarises the performance in terms of the reduction in dew points achieved by the various icing inhibitors tested at 0.13% by weight concentration in the same aviation fuel. Table 3 compares the relative effects of using different concentrations of the same inhibitor:

**TABLE 2**

| Additive | Dew Point (°C) |
|---|---|
| None | -1 |
| EDGE | -1 |
| EDP | -4 |
| BGE | -5 |
| BDGE | -5 |
| SOLVENT 14* | -35 |
| PnB | -3 |
| dPnB | -1 |
| PnBtert | -1 |

| | |
|---|---|
| * according to the present invention | |

**TABLE 3**

| Additive | Concentration (%) by wt | Dew Point (°C) |
|---|---|---|
| None | - | 0 |
| BGE | 0.1 | -2 to -3 |
| | 0.2 | -10 to -11 |
| BDGE | 0.1 | -2 to -3 |
| | 0.2 | 10 to -11 |
| | 0.25 | -13 to -14 |
| Solvent 14* | 0.1 | -14 to -35 |
| | 0.2 | -42 to -45 |
| | 0.4 | -45 to -47 |

| | | |
|---|---|---|
| * - according to the present invention | | |

A feature of the present invention is that there is basically no waste disposal problem since there is no separation or accumulation of fuel immiscible components and in view of this there is no need for emptying or cleaning the storage tanks on a regular basis.

## Claims

1. An icing inhibitor for hydrocarbon fuels contaminated with water said icing inhibitor comprising a polyethyleneglycol monoalkyl ether of the generic formula:
R-(OCH₂.CH₂)_{*n*}-OH (I)
wherein R is a C4-C6 alkyl group and *n* has a value from 3 to 8, said inhibitor being substantially free of components immiscible with said fuel.

2. An icing inhibitor according to Claim 1 wherein the polyethyleneglycol monoalkyl ether (I) (hereafter referred to as "PGME" for convenience) is an ether in which the alkyl group R is a C4 alkyl group and the *n* has a value of 3-4.

3. An icing inhibitor according to Claim 1 or 2 wherein the alkyl group R is an n-butyl group.

4. An icing inhibitor according to any one of the preceding Claims 1-3 wherein the PGME is a triethyleneglycol mono-n-butyl ether (also known as butyl triglycol ether and hence will hereafter referred to as "n-BTGE" for convenience).

5. An icing inhibitor according to any one of the preceding Claims wherein the PGME is used as a single ether or as an admixture thereof with other alkyl mono-, alkyl di- or alkyl polyglycol ethers.

6. An icing inhibitor according to Claim 5 wherein the admixture of glycol ethers contains a butyl triglycol ether.

7. An icing inhibitor according to Claim 6 wherein the the n-butyl triglycol ether is n-BTGE which is present as the major component in said admixture.

8. An icing inhibitor according to Claim 7 wherein the n-BTGE is present in the admixture in an amount of at least 60% by weight of the total admixture.

9. An icing inhibitor according to any one of the preceding Claims 5-8 wherein the admixture of glycol ethers comprises a butyl triglycol ether, and at least one alkyl di-, alkyl tetra- or alkyl penta-glycol ether.

10. An icing inhibitor according to any one of the preceding Claims 5-9 wherein the admixture of glycol ethers comprises n-BTGE and n-butyl tetra ethyleneglycol ether.

11. An icing inhibitor according to any one of the preceding Claims wherein said inhibitor comprises an admixture of the following components in approximate weight %:
| | |
|---|---|
| n-Butyl triglycol ether - | 75 |
| n-Butyl diglycol ether - | 2.5 |
| n-Butyl tetraglycol ether - | 19.0 |
| n-Butyl pentaglycol ether - | 2.0 |

12. An aviation fuel system comprising a hydrocarbon fuel contaminated with water, and an ice inhibiting amount of a polyethyleneglycol monoalkyl ether (I) as defined in any one of the preceding Claims 1-11.

13. An aviation fuel system according to Claim 12, wherein the icing inhibitor comprises a polyethyleneglycol monoalkyl ether (I) and is substantially free of components immiscible with said fuel.

14. An aviation fuel according to Claim 12 or 13 wherein the hydrocarbon fuel is selected from aviation and jet engine fuels which comprise a blend of hydrocarbons boiling suitably in the range from about 37°C to about 375°C.

15. An aviation fuel according to any one of the preceding Claims 12-14 wherein the hydrocarbon fuel comprises a blend of components boiling in the range from 90°C to 330°C.

16. An aviation fuel according to any one of the preceding Claims 12-15 wherein the hydrocarbon fuel comprises a blend of gas oils, kerosines and gasoline.

17. An aviation fuel according to any one of the preceding Claims 12-16 wherein the hydrocarbon fuels have an aromatic content ranging from 5 to 90 percent liquid volume of aromatics.

18. An aviation fuel according to any one ofthe preceding Claims 12-17 wherein the hydrocarbon fuel is selected from the group consisting of JET A, JET A-1, AVTUR, JP-3, JP-4, JP-5, JP-8 and jet kerosine.

19. An aviation fuel according to any one of the preceding Claims 12-18 wherein the icing inhibitor is present in said fuel in an amount ranging from 0.01 to 1% by weight of the hydrocarbon fuel.

20. An aviation fuel according to any one of the preceding Claims 12-19 wherein the icing inhibitor is present in said fule in an amount ranging from 0.1 to 0.5% by weight.
